

Nov. 12, 1968

W. H. HOGE

3,410,711

TRANSFER SHEET AND COPY SHEET SYSTEMS AND METHOD OF MAKING

Filed Nov. 22, 1963

FIG. 1



FIG. 2



FIG. 3



FIG. 5



INVENTOR  
William H. Hoge  
BY *Parsons, Clapp & Judd*  
*Master Taylor and Adams*  
ATTORNEYS

1

3,410,711

**TRANSFER SHEET AND COPY SHEET SYSTEMS  
AND METHOD OF MAKING**William H. Hoge, Rumford, Maine, assignor to Oxford  
Paper Company, New York, N.Y., a corporation of  
MaineFiled Nov. 22, 1963, Ser. No. 325,624  
15 Claims. (Cl. 117—36.1)

This invention relates to a system of coated papers for manifolding use. The invention includes transfer papers having a transferable coating on one side thereof capable of being transferred to a receiving surface by application of a pressure such as by a ballpoint pen, stylus, pencil or typewriter key, in the selective areas to which the pressure is applied. The invention includes manifold systems in which one or more sheets of paper having a pressure transferable coating adhered to one side thereof is used in combination with one or more sheets of paper having a specially prepared image receiving surface or receptor coating adhered thereto. The invention also includes receptive papers which are very economical in cost and which add to the quality of the transfer papers and the manifolding system.

Single or multiple copies of letters, invoices, shipping orders, account statements, and so forth are generally prepared today by using ordinary carbon paper interleaved between the original and the copy papers and the image transfer from the carbon paper transfer layer to the copy papers by applying writing pressure to the original paper.

Single and multiple copies have also been made without inserting the usual sheets of carbon paper between the copy sheets which are to receive images made by application of pressure hand or machine. Such systems generally comprise an original sheet having a transfer coating applied to the underside thereof and one or more copy sheets having image receiving surfaces coated on the top side and a transfer coating on the underside. Copies are made by applying pressure in a localized area to the top side of the original and the coating on the underside thereof transferred in the localized areas to the receiving surfaces of the copy papers in contact with the transfer coatings on the original and copy sheets.

Ordinary carbon paper is essentially composed of a paper base to which a transfer coating is applied to one side thereof and is usually composed of waxes, oils, suitable coloring pigments or dyes which are generally black but may be another color. The use of carbon paper involves the inconvenience of handling the separate sheets of paper. Conventional wax-oil transfer coatings are not commercially used on the back surfaces of the copy paper since the carbon transfer layer will smear and soil the hands and clothing of people handling the original or copies as well as transfer to other papers and surfaces that happen to come into contact with the transfer coating during normal use.

Attempts to formulate and produce multiple copy systems without inserting the usual sheets of carbon paper between these copy sheets by applying a transfer coating to the underside of the original and copy sheets have not achieved, to date, any great degree of commercial success. One of the few types of papers on the market today utilizes a type of system which involves a chemical reaction between an imbedded or encapsulated chemical in the transfer coat and a second ingredient applied to the topside of the copy paper. In this type of system, when pressure is applied to the top of the original, it releases a chemical contained in the transfer coating and transfers it to the copy paper and a reac-

2

tion takes place in the area of applied pressure to delineate the desired image.

These chemical reaction types of reproduction papers are costly and the number of copies which can be reproduced by conventional mechanical writing pressure has been rather seriously limited. They all seem to be based on dye systems which form light blue images which are unsatisfactory for optical scanning machines and which cannot be used with certain types of photocopy machines. The papers cannot be calendered after coating without prematurely releasing the chemicals and this prevents their use in smooth, dense calendered papers which will give the maximum number of copies. The chemical reaction papers also have problems in odor and fading.

Attempts to formulate and produce manifolding systems involving the application of a transfer coating to the reverse side of the original and copy papers have not been significantly successful for one or a combination of reasons. Most attempts to produce a paper having a transfer coating on the reverse side thereof have resulted in coatings which are not sufficiently smudge-proof. Such a coating will transfer easily to the hands of the user or to other papers or surfaces it comes into contact with under normal use and handling. Such transfer coatings generally have an oily or waxy appearance in feel and are not dry.

Attempts to overcome and improve the smudging properties of such papers have resulted in poor image transfer to the copy paper or receiving surface. In some cases, the transfer image is fragmented or quite hazy in appearance, and, therefore, very difficult to read and hard on the eyes. This is especially true when more than two or three copies are being made. In other cases, the transfer coating is too difficult to transfer by means of ordinary writing pressure by machine or hand resulting in light images which are also difficult to read as well as seriously limiting the number of copies which can be made. Further disadvantages of prior papers include instability to aging with moisture and/or heat resulting in a complete loss of the transfer properties of the transfer coatings or seriously diminished transfer properties.

The inability of prior reproduction papers having a transfer coating on one side thereof to go through normal and conventional printing processes without removal of portions of the transfer coating and gumming-up of the printing press has also been a serious problem. Other disadvantages of prior products include the necessity of high coat weight or special types of coatings which are costly, dusting of the transfer coating as well as poor adherence of the coatings to the paper base and generally poor paper characteristics. Inability of the receiving surface to adequately hold the image has also been a problem.

55 This invention broadly involves a base sheet, preferably paper, having a transfer coating adhered to one side thereof which is capable of being transferred from the surface of the base sheet to a special receptive surface by application of pressure to the reverse side of the paper and in which the transfer coating comprises a synthetic resinous adhesive having a glass transition temperature below about 40° C., and an inorganic pigment composed predominantly of platelets and in which the amount of adhesive is at least about 2% by weight based on the weight of the pigment.

60 The image receiving surface according to this invention comprises a synthetic resinous adhesive having a glass transition temperature below about 40° C. and which is essentially non-tacky to the casual finger touch but which when compressed against the transfer coat by ordinary hand or machine writing pressure develops sufficient

tack or adhesive affinity to remove transfer coat from the overlying surface.

In the drawing,

FIG. 1 shows a paper base having a transfer coating composed of an adhesive having a glass transition temperature below about 40° C. and platelets-type pigments;

FIG. 2 shows a paper base having a receptor coating adhered thereto, having a glass transition temperature below about 40° C.;

FIG. 3 is a view showing the original paper having a transfer coating on the reverse side thereof and a second paper base having a receptor, or image receiving surface coating adhered thereto;

FIG. 4 shows a manifolding system in which the papers are stacked with the transfer coatings on one side of the paper base in contact with the receptor coatings also adhered on one side of a paper base. The intermediate two papers have a transfer coating on one side and a receptor coating on the other;

FIG. 5 shows a paper base having a planographic printing surface adhered to one side thereof and a transfer coating adhered to the other. The transfer coating is in contact with a receptor coating on a second paper base as shown in the drawing.

Various pigments can be used in the transfer coat according to this invention as long as they are predominantly of the platelet-type. Examples of pigments predominantly of the platelet-type include various clays, such as China clay, kaolin clay and talc. Various other types of pigments such as needle, cubicle and spherical types do not operate satisfactorily according to this invention when used as the sole pigment. Other types of pigments including the needle, cubicle and spherical as well as thermoplastic organic pigments, such as polystyrene, can be substituted in part for the platelet-type pigments. The amount of such substitutions permissible, according to this invention, will, of course, vary not only with the type of platelet pigment used but with the type of needle, cubicle or spherical pigment used. It is, therefore, not possible to set forth exact amounts of the various needle, cubicle or spherical type pigments which can be substituted in part for the platelet-type pigments but this could readily be determined by routine experimentation by those skilled in the art with respect to any particular pigment system.

The amount of adhesive which can be used to bind the pigments to form the transfer coating has been determined to be between about 2 and 15% by weight based upon the weight of the pigments. Generally, the use of about 3% by weight of the adhesive when using clay as the sole pigment has been found to be advantageous. The use of an adhesive in excess of about 15% by weight seriously diminishes the transfer properties of the coating while the use of adhesives below about 2% by weight does not result in sufficient bonding power of the transfer coating to the base. The particular adhesive content referred to above was determined by using a common base paper stock having no release coating thereon. Thus, the use of release coatings, which is possible but not necessary according to this invention, may vary the minimum and maximum amounts of adhesives as will be appreciated by those skilled in the art. The type of pigment used will also offset the amount of adhesive and the 12 to 15% adhesive level will be of importance only when there are large amounts of hard-to-bind pigments, such as certain needle shaped materials, with the clay.

Various bases can be used for both the transfer and receptor coatings including coated and uncoated base paper stock. Transfer coatings on plastic films give very sharp images. It is an advantage of this invention, however, that conventional base stock commonly used for coatings can be used without previous treatment to hold both the transfer and receptor coatings.

The pigments referred to above which can be used according to this invention in the transfer coating are not used to impart color to the transfer coating and it is

the combination of the particular type of pigments with the particular type adhesive in particular ratios which gives the transfer coating the characteristics of internal weakness and fracturing which control the ability to transfer. Ordinarily, these transfer coatings containing the platelet-type pigment will be white. It is, of course, possible to transfer a white image to a surface of contrasting color but it is advantageous to add a coloring material to the transfer coating which does not interfere with the transfer properties or the other advantageous properties of the transfer coating. This will permit the use of a white or substantially white receptor surface and the image transferred to the receptor surface will then be of contrasting color to the receptor surface and easily legible.

Various coloring materials can be incorporated into the coating compositions such as carbon black, red oxide, chromium oxide and phthalocyanine pigments. Examples of specific commercial type pigments which have been used include carbon blacks marketed by Columbian Carbon under the trade name Aquablak, red oxides marketed by the Harshaw Chemical Company under the trade name Aurasperse Red Oxide W3041, chromium oxides marketed by the Harshaw Chemical Company under the trade name Aurasperse Chromium Oxide Green W6017, phthalocyanine pigments marketed by the American Cyanamid Company under the trade names Calctone Blue G and Calctone Green G. Water-soluble dyes can also be used as coloring materials. An example of a water-soluble dye which can be used is one marketed by the Allied Chemical Company under the trade name Soluble Blue P.

The amounts of coloring material which can be used will vary quite widely depending upon the particular coloring material being used and the desired shade and depth of color in transfer coating.

In calculating the percent by weight of adhesive which can be used according to this invention, the calculation has been made with respect to the platelet-type or predominantly platelet-type pigment which is not basically used as a coloring material according to this invention. Since very little of the coloring material or pigment is required, this factor can be ignored to some extent. If, however, large amounts of a colored pigment are employed, this might very well alter the percent of adhesive used according to this invention, especially if the coloring material is one which is difficult to bind by adhesives.

The coat weights of both the transfer and receptor coating can be quite low according to this invention. The coat weight of the transfer coating should be sufficient so that a sharp deeply colored image can be transferred but not sufficiently high so that the transfer coating will lose its scuff resistance. Generally, a coat weight of between about 3 and 6 pounds per ream can be used according to this invention but, of course, it is advantageous to use a coat weight as low as possible from a cost standpoint. The coat weight of the receptor coating is preferably about 1-2 pounds per ream or below and only has to be of a sufficient coat weight so that it will adequately receive and hold the transferred image. Some compositions when applied at a coat weight of about 1 to 2 pounds per ream will not be sufficiently receptive and in which case higher coat weights should be applied which will possess the desired tack or receptive properties.

Both the transfer coating and the receptor coating can be coated on a suitable base, preferably paper, by any conventional coating process. No special coating procedures and no special mixing procedures of either the transfer coating composition or the receptor coating composition are required.

The transfer coating of this invention can be calendered or supercalendered by conventional calendering equipment without any significant loss of its advantageous properties and particularly without any significant loss of its transfer properties. The calendering of the transfer coating adhered to the base reduces the caliper of the sheet and imparts to it improved manifolding characteristics, improved

sharpness of image without significant degradation of image darkness or shade and more copies can thus be obtained than with an uncalendered manifolding system. Calendering also renders the transfer coating smooth and gives it a shiny appearance.

The calenderability of the transfer coating also permits a much more economical process to be employed where the transfer coating is to be adhered to the back side of a duplicating master which normally would be calendered. In many instances, it is very desirable when imaging a master such as a planographic printing plate to have one or more copies immediately available prior to sending the plate out to the printer for the production of the copies. This can readily be accomplished by using a planographic printing plate with a transfer coat on the back side, and placing behind it a receptive coated sheet with the receiving surface in contact with the transfer coating. The printing plate is imaged in the usual manner. Thus, by imaging the printing plate, a copy is simultaneously made.

Most duplicating masters, such as planographic plates, require calendering to insure smoothness and proper functioning for production of optimum quality copies. Conventional transfer coatings, however, particularly those of the wax type, cannot be calendered since they smear, come apart, foul up the calendering rolls or lose their transfer properties. Thus, with conventional type transfer coatings, it would be necessary to (1) place a planographic printing coating on to a suitable base such as paper, (2) then calender the planographic printing surface, (3) and finally send through a coater to apply the transfer coating opposite the planographic printing coating, dried and then rerolled.

Duplicating masters such as planographic printing plates having a transfer coating on the opposite side can be prepared, according to this invention more economically than using the above sequence. The planographic printing coating is applied to one side of the paper and a transfer coating is applied to the opposite side of the paper simultaneously or by means of a tandem coater which is capable of successively applying the two coatings without an intermediate rolling up of the paper. As a second and final step, the sheet with both coatings can be run through conventional calendering equipment. The calendering thus not only accomplishes the required calendering of the plate surface but also adds the advantages noted above with respect to the calendered transfer coating.

The particular type of planographic printing coating is not a part of this invention and any variously known planographic printing coating described in numerous patents and literature references can be used. Examples of planographic coatings which can be used include insolubilized polyvinyl alcohol and insolubilized carboxymethyl cellulose.

The adhesives used to form the transfer coatings should contain a significant quantity, such as 20% or more, of a resin with a glass transition temperature below about 40° C. The term "glass transition" refers to the characteristic change in polymer properties from those of a relatively hard, brittle, glassy material to those of a softer, more flexible material or vice versa as the temperature is raised or lowered through the glass transition temperature. An adhesive or polymer having a glass transition temperature below about 40° C. when coated on a suitable base such as paper will normally be readily deformable and probably slightly tacky if adequate coat weights are used.

The transfer coat has such a high proportion of clay-like platelets to cause it to be very dry and non-tacky, regardless of the glass transition temperature of the adhesive used. The purpose of the soft adhesive is to maintain a deformability and a plasticizing quality in the transfer coat. A transfer coating prepared from hard adhesives such as starch or casein could be used for transfer to a suitable receptor coating but it would have other disadvantages which would greatly reduce its value. The hard adhesives form transfer coatings which are brittle, they tend

to fragment off when the substrate paper is folded or flexed and they are too dusty for general use. However, in some cases it may be desirable to replace a portion of the flexible adhesive with small quantities of hard adhesives in order to give the coating mixture the viscosity or levelling characteristics which are sometimes required for optimum high speed coating machine operation. Care must be taken to maintain a low enough level of total adhesive to allow the transfer coat to be removed from its base and at the same time retain a sufficiently high level of flexible adhesive to obtain the desirable cleanliness and performance properties.

It is well known in the art of calendering printing papers that the dusting characteristics of any coating based on pigment and brittle adhesive can be improved by the addition of small amounts of fatty materials such as calcium stearate and the same principles apply to the transfer coat of this invention. The fluidity or softness of the adhesive also tends to give a very sharp, nonfragmented and non-hazy image.

The receptor coatings of this invention are formed of a soft resinous material having a glass transition temperature below about 40° C. with the pigmentation and coat weight controlled to produce a receptor coat which is essentially non-tacky to the finger touch but which has a tacky adhesive effect on the lightly bonded pigment particles in the transfer coat when the two coatings are pressed together. This very desirable blend of properties for the receptive coat can be obtained by the use of a soft, tacky resin which normally would be tacky to the finger touch and which normally could not be wound into a roll of paper without causing the successive plies to be blocked or glued together. The key to the control of these problems is the careful control of the thickness of the coating of the soft resin. It was found that extremely thin coatings of the soft tacky resins are not tacky to the finger touch, they do not cause blocking in the roll of paper, and they retain all of the affinity for the pigment in the transfer coating to give very good manifolding performance. The optimum coat weight for the receptor coat is in the range of 0.5 to 2 pounds per 3000 sq. ft., with a rough paper requiring slightly more and a very smooth paper slightly less.

The use of soft resins as receptor coatings in manifolding systems is old in the art but these prior papers were never of any commercial significance for several reasons. The soft resins could never be used because of the previously mentioned problems of the receptive coated paper blocking together in the roll. The slightly harder resins which did not cause blocking were not sufficiently receptive to be of commercial interest. These slightly harder resins could be used to a slightly better advantage by increasing the thickness of the receptive coating but this placed them at a severe economic disadvantage. In some cases the resinous receptor coatings were modified for greater receptivity and less tackiness through the addition of certain types of soft waxes but this gave a surface with very poor receptivity to printing inks and this prevented the commercial success of the product. The prior receptive coatings were always hindered by the fact that the transfer coatings tended to be waxy in composition and the resinous receptor coats had poor affinity for the wax. In contrast, the resinous receptor coatings have very excellent affinity for the lightly bonded clay-like pigment particles in the transfer coat formulated according to this invention. The extremely thin receptor coat of the soft tacky resins to prevent the paper from blocking in the roll, offer an economic advantage over the heavier coatings. The receptor coat of the invention also has very excellent affinity for conventional printing inks used in the business forms industry.

It may be advantageous, depending upon the particular adhesive used, to add a small amount of pigment to the receptor coating adhesives in order to impart whiteness or a color thereto. The pigments should be added in small amounts because they tend to increase the minimum work-

able thickness of the receptive coat. If the thicker and more expensive pigmented coating is desired, it can be used to give good results with the transfer coatings according to this invention. Excessive pigment causes a serious deterioration in the performance of the receptor coatings and it has been found that if the weight of the pigment exceeds about 60% of the total weight of the pigment-adhesive mixture, the receptivity is seriously impaired and even at that level of pigment, the coat weight of the receptor coat must be increased to obtain satisfactory performance.

Thus, the particular type of polymer or resinous material which can be used as the adhesive or in formulating the adhesive for both the transfer and receptor coating according to this invention is quite broad, so long as it is an adhesive or has adhesive properties for binding platelet-type pigments such as clays and talcs to themselves and to a suitable base such as paper and that the adhesives as a whole have a glass transition temperature below about 40° C. under normal humidity and temperature conditions under which the paper is to be used.

Examples of synthetic resinous materials which can be used according to this invention for the receptor coating or in the transfer coating include polybutadiene, poly-n-butylacrylate, poly-n-butylmethacrylate, poly-n-decylmethacrylate, polydimethylbutadiene, polyethyl acrylate, poly-2-ethylhexyl acrylate, polyethylene glycol iso-butyrate methacrylate, poly-n-hexadecylacrylate, poly-n-hexylmethacrylate, polyisobutyl acrylate, polyisobutylene, polyisoprene, polymethacrylate, poly-n-octylacrylate, poly-n-octylmethacrylate, poly-n-propyl acrylate, poly-n-propyl methacrylate, poly-n-tetradecyl acrylate, poly-n-tetradecyl methacrylate, urethane rubber, polyvinyl acetate, and so forth. Various other adhesives can also be used as will be apparent to those skilled in the art.

There are also a number of other synthetic polymeric resinous adhesives which possess a glass transition temperature above about 40° C. which can be treated by the addition of plasticizing agents so that the adhesive as a whole will possess a glass transition temperature below about 40° C. Polyacrylic acid is an example of such an adhesive. Although this adhesive has a glass transition temperature above 40° C., films formed therefrom are hygroscopic and under normal conditions of humidity and temperature under which the transfer paper or receptor coating will be used, the film will take on water which will plasticize the film rendering it flowable and soft and will possess a glass transition temperature under such conditions below about 40° C. Examples of other adhesive materials having a glass transition temperature above 40° C. which can be lowered by the addition of plasticizing agents include polyacrylonitrile, cellulose acetate, cellulose nitrate, polyethylene glycol dimethacrylate, polyethylene glycol terephthalate, polyisopropyl methacrylate, poly-tertiary butyl acrylate, polytertiary butyl methacrylate, polymethyl methacrylate, polyvinyl alcohol, polyvinyl butyral, polyvinyl chloride-acetate, polyvinyl pyrrolidone, and so forth. Adhesives or polymers having a glass transition temperature about 40° C. can, of course, be substituted in part for the adhesives having a glass transition temperature below about 40° C. so long as the combination of the material results in a total adhesive which possess a glass transition temperature below about 40° C.

The transfer coating of this invention has the particular advantage of requiring no oily, waxy, fatty, greasy, migratory or evaporatable materials for satisfactory performance. These additions, used in customary transfer coatings result in bleeding of dyes from transfer coatings or adjacent surface coatings, penetration of coating materials into or through the paper, or evaporation of materials from the coating which would alter the properties of the transfer coating to cause poor aging properties. This is particularly important if the transfer coating is to be used to be placed on the reverse of a paper planographic printing plate, which is easily damaged by migratory plasticizers and oils. Thus, although there is described above

the possibility of altering some adhesive materials by, for example, the addition of plasticizers, the additive agents should be carefully selected and the amounts thereof limited to preserve as much as possible the advantageous properties of the transfer films of this invention. Plasticized adhesives can be used in either the transfer coat or in the receptor coat of this invention so long as the plasticized resin systems retain the previously described properties required for functionality and the shelf like stability and non-migrating characteristics required by the end use application.

It has also been found that the papers prepared according to this invention have a major advantage over previously produced papers of this type in the fact that there is no apparent loss in copying quality if they are used at higher temperatures, such as 30 to 100° C. The transfer coating is essentially unchanged because its performance is dependent upon the network of inorganic pigment particles and this network is relatively insensitive to heat.

10 The receptive coating is a material which is naturally tacky and soft at room temperature as well as higher temperatures and the careful control of coating thickness required for satisfactory properties at room temperature also yields satisfactory properties at the higher temperatures.

15 20 25 Although adhesives having a glass transition temperature below about 40° C. can be used according to this invention the most advantageous adhesives are those which possess a glass transition temperature below about 20° C. If the adhesives have a glass transition temperature below about 20° C., the adhesive and the transfer coating will more definitely maintain the flowability and softness required by the adhesive in the transfer coating. Adhesives having a glass transition temperature between 20° and 40° C. can in most instances be utilized according to this invention but the possibility always exists that such resins under particular operating conditions may become too hard or brittle.

20 30 35 40 The adhesives or polymers thus used according to this invention are soft adhesives which coalesce at approximately room temperature. They possess high extensibility and can be stretched. They are viscous and flowable at the temperature and humidity conditions under which they are used.

35 40 45 The following working examples illustrate various coating formulations which can be applied to a standard base stock paper to produce the receptor coatings or receptor papers according to this invention:

|    | Coating Compositions                                          | Parts by Weight (Wet) | Parts by Weight (Dry) |
|----|---------------------------------------------------------------|-----------------------|-----------------------|
| 50 |                                                               |                       |                       |
|    | Example 1:<br>HT clay 60% solids.....                         | 50.0                  | 30                    |
|    | 60/40 styrene-butadiene copolymer emulsion at 48% solids..... | 50.0                  | 24                    |
| 55 | Example 2:<br>HT clay 70% solids.....                         | 50.0                  | 35                    |
|    | 60/40 styrene-butadiene copolymer emulsion at 48% solids..... | 91.0                  | 43.7                  |
|    | Water.....                                                    | 66.0                  | -----                 |
| 60 | Example 3:<br>HT clay 70% solids.....                         | 32.6                  | 22.8                  |
|    | Acrylic film forming emulsion at 48% solids.....              | 62.0                  | 28.5                  |
|    | Water.....                                                    | 40.4                  | -----                 |
| 65 | Example 4:<br>HT clay 60% solids.....                         | 21.8                  | 13.1                  |
|    | Water dispersible titanium dioxide 50% solids.....            | 8.8                   | 4.4                   |
|    | 60/40 styrene-butadiene at 48% solids.....                    | 45.5                  | 21.8                  |
|    | Water.....                                                    | 33.0                  | -----                 |
| 70 | Example 5:<br>HT clay 60% solids.....                         | 21.8                  | 13.1                  |
|    | Water dispersible titanium dioxide 50% solids.....            | 8.8                   | 4.4                   |
|    | Acrylic film forming emulsion 46% solids.....                 | 47.4                  | 21.8                  |
|    | Water.....                                                    | 31.0                  | -----                 |
| 75 | Example 6:<br>HT clay 60% solids.....                         | 21.8                  | 13.1                  |
|    | Water dispersible titanium dioxide 50% solids.....            | 8.8                   | 4.4                   |
|    | Acrylic film forming emulsion copolymer 46% solids.....       | 47.4                  | 21.8                  |
|    | Example 7:<br>HT clay 60% solids.....                         | 21.8                  | 13.1                  |

| Coating Compositions                                                  | Parts by Weight (Wet) | Parts by Weight (Dry) |    |
|-----------------------------------------------------------------------|-----------------------|-----------------------|----|
| Water dispersible titanium dioxide 50% solids                         | 8.8                   | 4.4                   | 5  |
| Butyl rubber emulsion polymer 56% solids                              | 20.6                  | 11.5                  |    |
| Polyterpene resin 50% solids                                          | 20.6                  | 10.3                  |    |
| Example 8:<br>Butyl rubber emulsion polymer 56% solids                | 20.6                  | 11.5                  |    |
| Polyterpene resin 50% solids                                          | 20.6                  | 10.3                  |    |
| Flue gas calcium carbonate                                            | 21.8-27.2             |                       | 10 |
| Example 9:<br>Acrylic self-cross-linking emulsion polymer 45% solids  | 20.0                  | 9.0                   |    |
| Water                                                                 | 20.0                  |                       |    |
| Example 10:<br>Acrylic self-cross-linking emulsion polymer 45% solids | 10.0                  | 4.5                   | 15 |
| Polystyrene emulsion 45% solids                                       | 10.0                  | 4.5                   |    |
| Water                                                                 | 20.0                  |                       |    |
| Example 11:<br>Acrylic self-cross-linking emulsion polymer 45% solids | 10.0                  | 4.5                   | 20 |
| Polystyrene emulsion 45% solids                                       | 10.0                  | 4.5                   |    |
| Cationic fatty acid condensate 6% solids                              | 1.5                   | .09                   |    |
| Water                                                                 | 10                    |                       |    |
| Example 12:<br>Acrylic self-cross-linking emulsion polymer 45% solids | 15.0                  | 6.75                  |    |
| Cationic fatty acid condensate 6% solids                              | 0.6                   | .036                  | 25 |
| Water                                                                 | 20                    |                       |    |
| Example 13:<br>Ubasol S-300 36% solids                                | 200                   | 72                    |    |
| Water                                                                 | 70                    |                       |    |
| Ammonium hydroxide at 28% solids                                      | 3.0                   | 0.84                  | 30 |
| Water                                                                 | 15                    |                       |    |
| Example 14:<br>60/40 styrene butadiene emulsion copolymer 48% solids  | 32.6                  | 15.0                  |    |
| Water                                                                 | 68.0                  |                       |    |
| Example 15:<br>Acrylic emulsion copolymer, 46% solids                 | 32.6                  | 15.0                  | 35 |
| Sodium alginate, 1% solids                                            | 34.0                  | 0.34                  |    |
| Water                                                                 | 34.0                  |                       |    |
| Example 16:<br>Polyvinyl acetate emulsion copolymer, 54% solids       | 27.8                  | 15.0                  |    |
| Butyl benzyl phthalate                                                | 5.0                   | 5.0                   |    |

The reference to percent solids in all of the above examples refers to the percentage of solids contained in an aqueous medium. The acrylic emulsion used in Examples 3 and 5 was acrylic emulsion marketed by Rohm & Haas under the trade name Rhoplex AC-33. The acrylic emulsion used in Examples 6 and 15 was one marketed by Rohm & Haas Company under the trade name Rhoplex B-5. The polyterpene resin used in Examples 7 and 8 was marketed by the Pennsylvania Industrial Chemical Corporation under the trade name Piccolyte S-70. The self-cross-linking emulsion used in Examples 9, 10, 11 and 12 was marketed by Rohm & Haas under the trade name Rhoplex K-3. The cationic fatty acid condensate used in Examples 11 and 12 was marketed by the American Cyanamid Company under the trade name Cyron.

The following working examples illustrate various coating formulas which can be applied to a standard base stock paper to produce the transfer coatings or transfer papers according to this invention:

| Coating Compositions                                  | Parts by Weight (Wet) | Parts by Weight (Dry) |
|-------------------------------------------------------|-----------------------|-----------------------|
| Example 17:<br>HT clay 60% solids                     | 50-58                 | 30-35                 |
| 60/40 styrene-butadiene 48% solids                    | 2.5-3.0               | 1.20-1.44             |
| Carbon black 35% solids                               | 2.0-3.0               | 0.70-1.06             |
| Water                                                 | 40-60                 |                       |
| Example 18:<br>HT clay 60% solids                     | 72.6                  | 43.6                  |
| Acrylic emulsion copolymer, 46% solids                | 1.8                   | 0.85                  |
| 60/40 styrene-butadiene copolymer emulsion 48% solids | 1.8                   | 0.86                  |
| Sodium alginate 1% solids                             | 3.0                   | 0.03                  |
| Aurasperse Red Oxide W 3041 64% solids                | 20.0                  | 12.8                  |
| Water                                                 | 1.0                   |                       |
| Example 19:<br>HT clay 60% solids                     | 72.6                  | 43.6                  |
| Acrylic emulsion copolymer, 46% solids                | 1.8                   | 0.85                  |

| Coating Compositions                                                                                | Parts by Weight (Wet) | Parts by Weight (Dry) |
|-----------------------------------------------------------------------------------------------------|-----------------------|-----------------------|
| 60/40 styrene-butadiene copolymer emulsion, 48% solids                                              | 1.8                   | 0.86                  |
| Example 20:<br>Aurasperse Chromium Oxide Green W-3017 63% solids                                    | 18.6                  | 12.6                  |
| Calcotone Green G Paste 20% solids                                                                  | 3.2                   | 0.64                  |
| Water                                                                                               | 1.0                   |                       |
| 72.6                                                                                                | 43.6                  |                       |
| 1.8                                                                                                 | 0.85                  |                       |
| 60/40 styrene-butadiene emulsion copolymer                                                          | 1.8                   | 0.86                  |
| Calcotone Blue G Paste 20% solids                                                                   | 12.0                  | 2.4                   |
| Water                                                                                               | 1.1                   |                       |
| Example 21:<br>HT clay at 60% solids                                                                | 47.7                  | 28.6                  |
| Soluble Blue P dye                                                                                  | 0.6                   | 1.7                   |
| Acrylic emulsion copolymer, 46% solids                                                              | 0.6                   | 0.27                  |
| 60/40 styrene-butadiene copolymer emulsion, 48% solids                                              | 1.7                   | 0.82                  |
| Water                                                                                               | 49.4                  |                       |
| Example 22:<br>HT clay 60% solids                                                                   | 305.0                 | 183.0                 |
| 60/40 styrene-butadiene copolymer emulsion, 48% solids                                              | 8.8                   | 4.32                  |
| Carbon black, 35% solids                                                                            | 37.0                  | 12.45                 |
| Sodium alginate, 2% solids                                                                          | 106.5                 | 2.13                  |
| Water                                                                                               | 170                   |                       |
| Example 23:<br>Lamp black, dry                                                                      | 3.2                   | 3.2                   |
| HT clay, dry                                                                                        | 47.6                  | 47.6                  |
| Polystyrene resin of estimated molecular weight of 350, with melting point (ball and ring) of 50° C | 6.0                   | 6.0                   |
| Hydroxylecithin                                                                                     | 0.7                   | 0.7                   |
| Methyl Ethyl Ketone                                                                                 | 40.0                  |                       |
| Toluene                                                                                             | 20.0                  |                       |

The acrylic film forming emulsion copolymer used in Examples 18, 19, 20 and 21, was marketed by Rohm & Haas Company under the trade name Rhoplex B-5. The carbon black in Examples 17 and 22 was manufactured by Columbian Carbon Company under the trade name Aquablak B. The Aurasperse Red Oxide and Aurasperse Chromium Oxide were red and green pigments marketed

40 by the Harshaw Chemical Company. The Calcotone Green G and the Calcotone Blue G were phthalocyanine pigments marketed by the American Cyanamid Company under the above names. The water soluble Blue P was marketed by the Allied Chemical Company under that 45 trade name. The polystyrene resin in Example 23 was marketed by the Pennsylvania Industrial Chemical Corporation under the name of Piccolastic A-50.

Transfer coatings or transfer papers were also made in a similar manner to that set forth above employing an 50 HT clay water dispersion as a pigment and carbon black as the coloring matter and using as adhesives a mixture of 60/40 styrene-butadiene copolymer emulsion and a styrene-butadiene copolymer in which the styrene-butadiene copolymer was present at about 1.11% and the styrene maleic anhydride copolymer was present at about 3.86% by weight based on the weight of the clay. 55 Polyvinyl methyl ether-maleic anhydride was also substituted for the styrene maleic anhydride copolymer in the same weight percentage as the styrene maleic anhydride copolymer.

Example 14 shows the production of two separate transfer coatings, one in which the styrene-butadiene was 2.5 percent, and carbon black 2.0 percent and the other 3.0 percent styrene-butadiene and 3.0 percent carbon black.

The transfer coating formulations set forth in the above examples were all coated on one side of a conventional untreated paper web base between about 2 and 5 lbs. per ream and dried. The reverse side of the paper base web 70 was coated with the receptor coating formulation of Example 15 at a coat weight of between about 0.5 and 2 lbs. per ream and dried. The resulting web was cut into sheets which had a transfer coating on one side and a receptor coating on the other.

The transfer coatings were essentially dry and smudge-

proof and had no oily or waxy appearance or feel, would not rub off onto other papers or onto hands during normal use or handling, and those papers having the transfer coating and/or the receptor coating adhered thereto had good paper characteristics and good handling characteristics.

The receptor coatings were printed upon by conventional printing processes and the printing characteristics were excellent. The printing of the receptor surface of the papers with a transfer coating on the back also exhibited excellent printing characteristics without interference of the function of the transfer coating and the transfer coating did not come off during the printing process, or in any manner foul up the printing press.

The sheets of paper having the transfer coating on one side and the receptor coating on the other were assembled in the same manner as shown in FIG. 4 but using ten sheets in the same type combination instead of the four shown in the drawing. The first paper had a receptor coating on top and the last paper had a transfer coating on the bottom.

Writing pressure by means of a typewriter was applied to the top paper and that portion of the transfer coating corresponding to the selected area of applied pressure by the typewriter keys readily transferred to the receptor coatings reproducing the image pressed on the top paper as shown in FIG. 3. In all cases, a legible image was produced on the tenth sheet. The images produced especially on the first five copy sheets, were sharp, unfragmented, had a dense color and were easily and readily legible. The image received on the receptor coating was not smeared through normal handling of the copy paper.

Similar tests on sets of five copy sheets showed that any of the transfer coatings as set forth in Examples 17-23 give good quality copy with any of the receptor coatings set forth in Examples 1-16. All tests resulted in substantially the same results as referred to above with respect to the use of the transfer coatings when used in conjunction with the receptor coating set forth in Example 15.

Although the transfer coatings can be transferred by means of writing pressure to ordinary papers of the various kinds in use today, the combination of the transfer papers of this invention with the receptor papers of this invention is particularly advantageous. The specificity of transfer of the transfer coatings to the receptor coatings results in the production of a much clearer, darker and sharp image than would be obtainable with ordinary papers. In addition, the transfer coatings are much easier to transfer by means of writing pressure to the receptor coatings and thus many more legible copies can be produced by using the receptor coating of this invention than would be possible with ordinary papers. This specificity of transfer of the transfer coatings to the receptor coatings does not, however, interfere with the smudge-proofness of the transfer coating and the transfer coating will not be transferred accidentally or scuff off onto other papers during ordinary handling thereof nor will it transfer to or scuff off onto the receptor coating thereon during normal use or handling. In spite of this smudge-proofness of the transfer coating toward the receptor coating during ordinary handling, the transfer of the transfer coating to the receptor coating by means of writing pressure was excellent. The transfer coatings, as well as the receptor coatings of this invention, were clean, not dusty and the adherence of the coatings to the paper base was also very good.

A suitable paper base was coated with a transfer coat as set forth in Example 17 and calendered by conventional calendering techniques. No difficulties were encountered during the calendering of the transfer coating and after the transfer coating was calendered, it was subjected to similar tests as set forth above. No reduction in the transferability of the transfer coat to the receptor coat was observed nor was any degradation of the quality

of the image observed over the non-calendered sheets. In fact, the transfer of the image was improved when applied to the receptor coatings probably due to the reduction in the caliper of the sheets and the smoothness of the transfer coating. The specificity of the transfer coating to the receptor coating when compared with ordinary papers in common use was even more pronounced with the calendered sheet than with the uncalendered sheet. In other words, the transfer of the image to the receptor coatings of this invention using a calendered transfer coating was not degraded with respect to transfer of the coatings or quality of the image while it became significantly more difficult to transfer an image from the calendered transfer coatings to ordinary paper. The calendered transfer coating was also more smooth and shiny and thus was better looking and also had a better feel and paper characteristic in general. The calendered transfer coating was even more smudge-proof than the uncalendered transfer coating.

A suitable paper base was coated with a planographic printing surface comprising insolubilized polyvinyl alcohol as known in the art on one side and the other side coated with the transfer coating formulation of Example 17. The dried coatings were then simultaneously calendered by conventional techniques without difficulty. The planographic surface was then imaged in the conventional manner with a receptor sheet in contact with the transfer coating and an excellent copy of the imaged plate obtained thereon. The plate was then placed on an off-set press and copies produced in the conventional manner without difficulty or any apparent degradation of the plate surface or interference with the printing process.

All of the above transfer coatings were applied to the paper bases at a coat weight of between 3 and 6 pounds per ream and all of the above receptive coatings were applied to the paper base at a coat weight of between about 0.5 and 2 pounds per ream. A ream, as used in this disclosure, is approximately 3000 square feet of paper.

I claim:

1. A manifolding system comprising a base sheet having a transfer coating on one side thereof and a base sheet having a receptor coating on one side thereof and in which the receptor coating is in contact with the transfer coating, said transfer coating comprising predominantly finely divided inorganic platelet-type particles bound together and to the base sheet by between about 2 and 15% by weight adhesive based on the weight of the platelet-type particles and in which the adhesive contains at least about 20% by weight an adhesive having a glass transition temperature below about 40° C. and which is of a nature to yield a lightly bonded flexible transfer coating, said receptor coating comprising a soft resinous plastic film-forming adhesive having a glass transition temperature of less than about 40° C. and applied to the sheet at a sufficiently low coat weight so that it is not tacky to the normal finger touch and does not exhibit blocking characteristics in roll form.

2. The manifolding system of claim 1 in which the receptor coating is applied to the sheet at a coat weight of between about 0.5 and 2 pounds per 3,000 square feet.

3. The manifolding system of claim 1 in which the adhesive contains at least one member of the group consisting of styrene-butadiene copolymers, acrylic polymers and acrylic copolymers.

4. The manifolding system of claim 2 in which the transfer coating pigment is clay.

5. The manifolding system of claim 3 in which a coloring material is present in the transfer coating.

6. A receptive coated paper for receiving an image transferred to said coating from a transfer coating containing predominantly platelet-type inorganic pigments by means of writing pressure comprising a base paper having a coating adhered to one side thereof at a coat weight of between about 0.5 and 2 pounds per 3,000

square feet of paper depending upon the smoothness and porosity of the base paper, said coating comprising a soft resinous plastic film-forming adhesive having a glass transition temperature below about 40° C. which would normally be tacky to the touch and have blocking characteristics in a paper roll if applied to the paper at a coat weight above about 2 pounds per 3,000 square feet but when applied to the paper between about 0.5 and 2 pounds per 3,000 square feet is not tacky to the normal finger touch and has a strong affinity to said transfer coating containing predominantly platelet-type pigments.

7. The receptive coated paper of claim 6 in which the adhesive contains at least one member of the group consisting of styrene-butadiene copolymers, acrylic polymers and acrylic copolymers.

8. The receptive coated paper of claim 6 in which the coating contains between about 0 and 125% by weight of an inorganic pigment based on the weight of the resin.

9. A copy paper having a transfer coating adhered to one side thereof and which is capable of being transferred from the surface of the paper to a receiving surface by application of writing pressure to the opposite side opposite the adhered transfer coating, said transfer coating comprising predominantly finely divided inorganic platelet-type particles bound together and to the base paper by between about 2 and 15% by weight adhesive based on the weight of the platelet-type particles and in which at least about 20% by weight of the adhesive has a glass transition temperature below about 40°C. to produce a lightly bonded flexible transfer coating and in which the transfer coating is calendered.

10. The method of manufacturing copy paper having a transfer coating adhered to one side thereof which is capable of being transferred from the surface of the paper to a receiving surface by application of writing pressure to the side opposite the adhered transfer coating which comprises applying to the base paper sheet a coating composition comprising finely divided inorganic particles predominantly of the platelet-type and between about 2 and 15% by weight adhesive based on the weight of the platelet-type particles and in which at least 20% by weight of the adhesive has a glass transition temperature below about 40°C., drying coating to produce a lightly bonded transfer coating, and calendering the transfer coating.

11. The method of manufacturing a duplicating master comprising a base having a transfer coating on one side

thereof which comprises applying to one side of the base a duplicating master coating, applying to the other side of the base a transfer coating comprising finely divided inorganic particles predominantly of the platelet-type of between about 2 and 15% by weight adhesive based on the weight of the platelet-type particles and in which at least about 20% by weight of the adhesive has a glass transition temperature below about 40°C., drying the coatings and simultaneously calendering the duplicating master coating and the transfer coating.

12. The method of claim 11 in which the duplicating master coating is a planographic coating.

13. A duplicating master having a duplicating master coating adhered to one side thereof and a transfer coating adhered to the other side thereof, said transfer coating comprising finely divided inorganic particles predominantly of the platelet-type and between about 2 and 15% by weight adhesive based on the weight of the platelet-type particles and in which at least about 20% by weight of the adhesive has a glass transition temperature below about 40°C. and having both the duplicating master coating and the transfer coating calendered.

14. The duplicating master of claim 13 in which the duplicating master coating is a planographic printing plate coating.

15. A copy paper having a transfer coating adhered to one side thereof and which is capable of being transferred from the surface of the paper to a receiving surface by application of writing pressure to the opposite side opposite the adhered transfer coating, said transfer coating comprising finely divided inorganic particles predominantly of the platelet-type bound together and to the base paper by between about 2 and 15% by weight adhesive based on the weight of the platelet-type particles and in which at least about 20% by weight of the adhesive has a glass transition temperature below about 40°C. to produce a lightly bonded, flexible transfer coating.

#### References Cited

##### UNITED STATES PATENTS

|           |        |           |       |          |
|-----------|--------|-----------|-------|----------|
| 627,229   | 6/1899 | Foster    | ----- | 117—36.3 |
| 1,845,568 | 2/1932 | Strawn    | ----- | 117—36.3 |
| 2,970,931 | 2/1961 | Gumbinner | ----- | 117—36.1 |
| 3,169,880 | 2/1965 | Strauss   | ----- | 117—36.3 |
| 3,186,861 | 6/1965 | Smith     | ----- | 117—36.1 |

MURRAY KATZ, Primary Examiner.